

## UNITED STATES PATENT OFFICE

2,423,450

PREPARATION OF SYNTHETIC ORGANIC  
DETERGENT PARTICLES HAVING ONLY  
SLIGHT DUST-FORMING TENDENCIES

Robert Franklin Heald, Nutley, and Minor Leslie Givan, East Orange, N. J., assignors to Colgate-Palmolive-Peet Company, Jersey City, N. J., a corporation of Delaware

No Drawing. Original application April 17, 1941, Serial No. 388,989. Divided and this application September 28, 1943, Serial No. 504,160

4 Claims. (Cl. 252—161)

1

The present invention relates to a process of treating synthetic detergents and, more particularly, to a process of preparing water-soluble non-fatty acid soap organic detergents, especially those of the type of organic sulphates and sulphonates, in sprayed, granulated and chip form to reduce dust therein, and to the product of such process.

Spray-dried detergents have been employed for both industrial and domestic uses for many years, because of their relative ease of solution due to the large surface area exposed. Detergents in chip and granulated form have similarly been used for the same reason. Up to the advent of the present invention there were attendant disadvantages in the use of these materials which considerably limited their employment. Because of their reduced size, there is always associated with the product an appreciable portion of fines, which causes a dust nuisance. This dust is objectionable both from the standpoint of cleanliness and because it acts as an irritant upon the mucous membrane of the user.

In seeking a method for eliminating these disadvantages, the prior art has suggested reducing the proportion of fines. This was, at best, an expensive operation, and it was found, moreover, that the removal of fines in any practical degree had little effect upon the amount of dust raised in the use of these synthetic detergent particles. This was due to the fact that the most troublesome or irritating dust is produced by the disintegration of the coarser particles during normal handling, resulting in a particularly fine powder, very small in percentage but very objectionable because of fineness and number of particles. Although this problem is an old one in the industry and although many suggestions and proposals have been made for solving it, none, so far as is known, has given a satisfactory solution upon a practical and industrial scale.

It is an object of the present invention to provide an improved process for treating synthetic detergents, during the manufacture of said detergents in sprayed, granulated and chip forms, to reduce dust therein, whereby detergent particles having greatly reduced irritant effect in use are produced.

It is also an object of this invention to provide a process for preparing detergents of the type of organic sulphates and sulphonates in particulate form having only slight dust-forming tendencies.

Another object of the invention is to provide 55 any of the manners described to synthetic deter-

2

particles of a synthetic detergent having greatly reduced dust-forming tendencies.

The invention further provides beads and grains of synthetic detergents of the type of organic sulphates and sulphonates having high washing efficiency and at most only slight dust-forming tendencies.

Other objects and advantages of the present invention will be apparent to those skilled in the art from the following description.

Broadly stated, according to the present invention, the addition of a relatively small proportion of a petroleum oil fraction to a synthetic detergent results in a composition having considerably less tendency to form dust. A remarkable feature of the invention is that the addition of the oil has little or no effect upon the washing efficiency. The incorporation of mineral oil is particularly advantageous in the manufacture of spray, granulated and chip detergents of the type of organic sulphates and sulphonates. One method of adding the oil in making the improved detergent beads and grains of the invention comprises spraying the detergent in fluid (i. e., liquid or plastic) form into an air stream in a tower in a procedure commonly employed in the art and passing the resulting beads and/or grains to a cooling chamber in the usual manner, and then spraying oil upon the detergent particles 25 during the cooling operation. This method of incorporating the mineral oil by spraying is also employed in reducing the dust otherwise occurring in a detergent product resulting from the granulation of a mechanical mixture of detergent 30 chips or flakes and dry builders. In general, in the manufacture of synthetic detergent products other than mechanical mixes, the mineral oil may be added in bulk to the detergent material before it is dried, as this method is cheaper and 35 more convenient. Thus, the addition of the mineral oil to the crutcher mix requires no greater proportion of oil and, in general, also yields satisfactory results.

The present process is applicable to the treatment of various water-soluble, non-fatty acid soap, organic detergents, such as the salts of organic sulphates and sulphonates, with or without any of the builders or fillers usually employed by the art. A preferred product comprises the 45 sodium salt of sulphated coconut oil fatty acid monoglyceride as the active ingredient. Other detergents suitable for treatment include salts of sulphonated and sulphated long-chain fatty alcohols. Thus, mineral oil can be added in 50 sodium salt of sulphated coconut oil fatty acid monoglyceride as the active ingredient. Other detergents suitable for treatment include salts of sulphonated and sulphated long-chain fatty alcohols. Thus, mineral oil can be added in

gents containing the sulphuric esters of oleyl alcohol, of lauryl alcohol or of primary stearyl alcohol, salts thereof, including sodium lauryl sulphate or the like, etc., to produce our novel compositions and to achieve the desirable results pertaining thereto and herein described.

In selecting a petroleum fraction for use in accordance with the invention, kerosene (astral oil), white mineral oil, and heavy mineral oils of various viscosities are especially suitable for reducing dust-forming tendencies when incorporated in the detergent. Of these, the higher fractions are somewhat more desirable in that smaller proportions of the oil can be used and that there is less odor. Specifications for suitable oils are as follows:

*Kerosene*

|                       |        |
|-----------------------|--------|
| A. P. I. gravity      | 46.0   |
| Flash point           | °F 127 |
| Initial boiling point | °F 350 |
| Final drop            | °F 536 |

*White mineral oil*

|                            |                |
|----------------------------|----------------|
| Specific gravity, 15.6°    | 0.845 to 0.855 |
| Viscosity Saybolt, 100° F. | sec 80 to 90   |
| Initial boiling point      | °F 572         |
| 90% distilled at           | °F 748         |
| Residue                    | per cent 10    |

*Heavy mineral oils*

|                                 | No. 1 | No. 2 | No. 3   | Per cent |
|---------------------------------|-------|-------|---------|----------|
| A. P. I. gravity                | 28.5  | 27.0  | 26.0    |          |
| Flash point, °F                 | 300   | 365   | 385     |          |
| Viscosity Saybolt, 100° F., sec | 75-80 | 205   | 300-315 |          |
| Initial boiling point, °F       | 568   | 609   | 597     |          |
| Final distillation point, °F    | 754   | 737   | 711     |          |
| Distilled, percent              | 95    | 80    | 40      |          |
| Residue, percent                | 5     | 20    | 60      | 100.0    |

Still higher boiling fractions, having Saybolt viscosities of more than 600 seconds, give very satisfactory results.

It is advantageous to employ oils with flash points high enough to avoid fire hazards, especially where the oil is incorporated in the detergent before spraying, as the high temperature of the spraying tower must be taken into consideration. In selecting the mineral oil, the viscosity of the oil is not of great effect, although slightly better results are obtained with oils of higher viscosity. This may be due, in part, to the fact that these oils in general represent higher fractions. If the oil is too viscous, it is difficult to handle and can therefore be inconvenient.

Using such oils as hereinbefore described, proportions of the mineral oil of about 0.5% to about 8.0% (on the basis of the finished product) reduce the dust-forming tendencies in synthetic detergent particles. When using oils of relatively high boiling fractions, about 0.5% to about 3.0% of oil is suitable, about 0.5% to about 1.5% of mineral oils of this type being preferred. This proportion decreases dust to a minimum, without affecting the detergent properties and handleability of the product. It will be understood that larger proportions of mineral oil must be employed where lighter fractions are used, and, in some cases, even several per cent, e. g., as much as about 2.5% to about 8%, are preferred for reducing dust to the considerable degree desired. Below the optimum proportion of mineral oil, of the preferred type, the best results are not obtained; above this proportion, the treated particles exhibit a certain stickiness, which is un-

desirable from the standpoints of both the consumer and the packager, and the detergency value of the product is deleteriously affected.

The following example is merely illustrative of the present invention, and it will be understood that the invention is not limited thereto.

*Example*

About 0.65 part of a heavy mineral oil (mineral oil No. 3) is added to 99.35 parts of an organic detergent solution in a crutcher. The detergent solution has the following composition, the active ingredient being the sodium salt of sulphated coconut oil fatty acid monoglyceride:

|                    | Per cent   |
|--------------------|------------|
| Water              | About 59.6 |
| Inorganic salts    | About 25.0 |
| Active ingredient  | About 13.3 |
| Unreacted material | About 1.4  |
|                    | 99.3       |

The materials are thoroughly mixed, and the mixture is passed to a spray tower for spraying in a usual manner.

Upon spray drying, about 59.2% of the crutched material is lost as moisture. The dried product gives the following analysis, the mineral oil showing up with any unreacted material:

|                          | Per cent   |
|--------------------------|------------|
| Moisture                 | About 1.0  |
| Inorganic salts          | About 61.4 |
| Active ingredient        | About 32.6 |
| Unreacted (raw material) | About 3.4  |
| Mineral oil              | About 1.6  |
|                          | 100.0      |

The results obtained according to the present invention are superior to those obtained by the prior art. Even where part of the fines in synthetic detergent particles has been removed by sizing, the dust raised with such material is much greater than with the oil-treated material of this invention.

The term "particle" used in the present specification and in the appended claims is intended to include sizes and shapes of material having at least one dimension of relatively low order, such as grains, beads, chips, flakes and other forms having proportionately large surface area. Similarly, the term "particulate" as applied to synthetic detergents is intended to include those forms having at least one small dimension. Particles having solid centres are usually referred to as "grains," while hollow particles are generally known as "beads." Grains and beads frequently occur together and are distinguishable from chips and flakes in that all of their dimensions are of relatively low order.

The present application is a division of our prior application Serial No. 388,989, filed April 17, 1941.

The present invention has been described with reference to illustrative examples and proportions, but it will be appreciated by those skilled in the art that other variations and modifications of our invention can be employed and that equivalents can be substituted therefor, without departing from the principles thereof.

We claim:

1. A process of preparing detergent particles which comprises forming particles of a synthetic organic non-soap water-soluble detergent of the class consisting of sulphates and sulphonates, and spraying said particles after formation with

about 0.5% to about 3% of a mineral oil fraction having an initial boiling point of about 350° F., said percentage being based upon the amount of mineral oil in the final product, whereby improved particles having only slight dust-forming tendencies are produced.

2. A process of preparing detergent particles which comprises spraying about 0.5% to 8% of a mineral oil fraction having an initial boiling point of at least about 350° F. upon preformed particles of a synthetic organic non-soap water-soluble detergent of the class consisting of sulphates and sulphonates, said percentage being based on the amount of mineral oil in the final product, whereby particles having reduced dust-forming tendencies are produced.

3. A process of preparing detergent particles having only slight dust-forming tendencies which comprises mixing a mineral oil fraction having an initial boiling point of at least about 350° F. with a synthetic organic non-soap water-soluble detergent of the class consisting of sulphates and sulphonates in fluid form, and then forming said mixture into particles, the amount of said oil being within the range of about 0.5% to 8% by weight of said particles.

4. A process of preparing detergent particles having only slight dust-forming tendencies which comprises mixing a mineral oil fraction having an initial boiling point of at least about 350° F. with a synthetic organic non-soap water-soluble

detergent of the class consisting of sulphates and sulphonates, and then spray drying said mixture, the amount of said mineral oil being within the range of about 0.5% to 8% by weight of the spray dried product.

ROBERT FRANKLIN HEALD.  
MINOR LESLIE GIVAN.

## REFERENCES CITED

10 The following references are of record in the file of this patent:

## UNITED STATES PATENTS

| Number       | Name           | Date           |
|--------------|----------------|----------------|
| 15 1,715,999 | Flammer et al. | June 4, 1929   |
| 2,016,289    | McGill         | Oct. 8, 1935   |
| 2,206,289    | McDaniel       | July 2, 1940   |
| 2,130,362    | Muncie         | Sept. 20, 1938 |
| 1,886,632    | Broeman        | Nov. 8, 1932   |
| 20 1,479,757 | Trent          | Jan. 1, 1924   |
| 2,296,121    | Smith          | Sept. 15, 1942 |
| 2,356,443    | Bissinger      | Aug. 22, 1944  |

## FOREIGN PATENTS

| 25 Number | Country       | Date          |
|-----------|---------------|---------------|
| 23,054    | Great Britain | 1894          |
| 447,521   | Great Britain | Dec. 28, 1937 |

## OTHER REFERENCES

|    |                                                                             |
|----|-----------------------------------------------------------------------------|
| 30 | Dyestuffs—Booklet of Allied Chem. & Dye Corp., N. Y., Sept. 1942, page 205. |
|----|-----------------------------------------------------------------------------|